

# UNITED STATES PATENT OFFICE.

JOHANNES KORSELT, OF ZITTAU, GERMANY, ASSIGNOR, BY MESNE ASSIGNMENTS, TO THE CHEMICAL FOUNDATION, INC., A CORPORATION OF DELAWARE.

## PROCESS FOR THE TREATMENT OF SILK WITH RESERVES FOR THE PURPOSE OF INCREASING ITS STRENGTH AND ELASTICITY.

1,318,339.

Specification of Letters Patent.

Patented Oct. 7, 1919.

No Drawing.

Application filed November 15, 1915. Serial No. 61,656.

*To all whom it may concern:*

Be it known that I, JOHANNES KORSELT, a citizen of the Kingdom of Saxony, Germany, residing at Zittau, in Saxony, have 5 invented certain new and useful Improvements in Processes for the Treatment of Silk with Reserves for the Purpose of Increasing Its Strength and Elasticity, of which the following is a specification:

10 This process relates to the treatment by reserves of silk with a view to increasing the strength and elasticity of the same. In accordance with this process silk is acted upon by organic compounds, particularly by 15 compounds containing nitrogen or sulfur and nitrogen combined and which are soluble in water or in dilute acids and which moreover, neither sublime at ordinary temperature nor are volatilized or vaporized 20 and which fail to yield any undesired color-reactions with metal salts (as for instance do thio-cyanates), such reagents being dissolved in suitable solvents, the temperature of which may be raised to boiling according 25 to requirements, and being made to act upon the silk material after loading the same, for instance according to the tin-phosphate-silicate process. It has been ascertained that in the operation of this process those organic 30 compounds particularly nitrogenous compounds or those containing nitrogen and sulfur, which are not volatilized by intense radiation of the rays of the sun and which cannot be removed from the silk fiber by a 35 strong draft of air, produce the most intense and most permanent reserve action upon the silk material.

In order that the solution of the reserve body may be adapted to more completely 40 permeate the fibroin which has become swollen and therefore ordinarily less permeable after loading, and in order to prevent the reserve from depositing merely upon the peripherous layers of the fibroin, it is advisable to carry on the treatment at such 45 temperature and for such length of time as to insure thorough impregnation.

In order to effect an additional fixation 50 of the reserve body in the interior of the silk fiber after impregnating, I may precipitate the reserve body in the interior of the fiber by means of well known reactions so as to make said reserve body insoluble or difficultly soluble, by means of which the

durability of the protecting action of the 55 reserve is further increased.

The substances employed according to my invention act in such a manner that they will protect silk which has been loaded by the tin-phosphate-silicate process, from being 60 decomposed or oxidized by oxygen or by oxygen carriers such as tin-compounds which liberate oxygen when decomposed. Of such substances I may mention by way of example, cholin, betaine, and alkaloids 65 generally and all those organic compounds which, when treated with loading agents, are more readily oxidized than fibroin. On the other hand, those substances which effect 70 merely a mechanical holding together of the broken down or brittle fibroin by means of their adhesive properties and which, according to their natural properties, are employed as mere sizing agents, as for instance glue, dextrin or "diastaphore". 75 are not comprised by my invention. On the contrary, the substances which are comprised by my invention are characterized by the fact that they change neither the touch nor the color and appearance of the 80 silk fiber. Furthermore my invention does not include those organic substances which are spontaneously decomposed by the loading agent and in the presence of the action of sun light without forming any decompo- 85 sition-products which have any practical efficiency as protecting or reserve agents, such as urea, or thio-urea, nor volatile substances, such as formaldehyde, hydroxylamin, and their salts or derivates, nor such 90 compounds as produce undesired color-reactions, such as the thio-cyanates or hydroquinone.

In carrying the process into effect I may proceed by treating the silk after loading 95 with a five percent-solution of cholin.

I may also proceed by treating the silk after loading with a two per cent solution of sodium-hippurate, then removing the liquid by centrifugal action, and depositing 100 the hippuric acid by means of hydrochloric acid within the fiber in a difficultly soluble state.

As compared with all processes heretofore known for the protective treatment of silk 105 a most important technical improvement is accomplished by my process on account of the universal applicability of all organic,

soluble, non-volatile, compounds of the kind hereinbefore referred to, which are more readily oxidized than fibroin, particularly nitrogenous or nitrogen and sulfur containing compounds.

5. What I claim is:—

1. The process for the protective treatment of silk; consisting in loading the silk by the tin-phosphate-silicate method, and 10 then treating the loaded silk with a non-volatile alkaloid that is more readily oxidized than fibroin and which will not decompose the silk fiber.

15. The process for the protective treatment of silk consisting in loading the silk by the tin-phosphate-silicate method, treating the silk thus loaded with a readily soluble nitrogenous compound containing nitrogen and sulfur which will not volatilize said tin 20 loading compound and at a temperature and for a sufficient length of time to effect a thorough permeation of the silk with the compound and without decomposition of the silk fiber, and precipitating the reserve body 25 in the interior of the silk by well known reactions.

2. The process for the protective treat-

ment of loaded silk, consisting in loading the silk by the tin-phosphate-silicate method, then treating the silk thus loaded with an 30 organic nitrogenous compound readily soluble in water which will not decompose the silk fiber, contains nitrogen and sulfur, is not volatile at an ordinary temperature and is readily oxidizable, to preserve the touch, 35 color and appearance of the silk and which will prevent deterioration of the silk by counteracting salts, and finally precipitating the reserve body in the interior fiber of the silk by well known reactions.

4. The process for the protective treatment of silk, consisting in loading the silk by the tin-phosphate-silicate method, then treating the loaded silk with cholin, and finally precipitating the cholin that has been 45 added to the silk and held within the fiber thereof by well known reactions.

In testimony whereof I have hereunto set my hand in presence of two subscribing witnesses.

DR. JOHANNES KORSELT.

Witnesses:

HENRY HASPER,  
ARTHUR SCHROEDER.